

Nov. 21, 1939.

J. L. COLLINS

2,180,798

ELECTROLYTIC DEVICE

Filed July 20, 1936



BY

INVENTOR.  
JOSEPH L COLLINS

Dorsey & Cole

ATTORNEYS

## UNITED STATES PATENT OFFICE

2,180,798

## ELECTROLYTIC DEVICE

Joseph L. Collins, North Adams, Mass., assignor  
to Sprague Specialties Company, North Adams,  
Mass., a corporation of Massachusetts

Application July 20, 1936, Serial No. 91,614

8 Claims. (Cl. 148—8)

My present invention relates to electrolytic devices, and more particularly to electrolytic condensers both of the so-called "wet" and so-called "dry" types.

5 To increase the surface area of the filming electrode and thus of the capacity of the condenser, it is known to subject the electrode to chemical etching prior to its film formation, and various etching processes and schedules are used for this 10 purpose, whereby a two- to six-fold increase in capacity is obtained, compared with condensers having unetched electrodes of the same dimensions.

15 However, in the manufacture of condensers having such etched electrodes, a serious difficulty arises, as the capacities of the individual condensers will vary within wide limits in spite of a most careful adherence to close manufacturing specifications and the use of aluminum of the 20 same origin, and such capacity variations may be of the order of  $\pm 25\%$  and more, whereas condensers using unetched electrodes can be conveniently manufactured within capacity tolerances of  $\pm 5$  to  $\pm 10\%$ .

25 The above wide-range variations in capacity, resulting with etched electrodes, have several contributing factors.

First, the filming metal used, which is usually aluminum, while of high purity still contains 30 about .1 to .3% of impurities, and aluminum sheets or foils obtained from different ingots and even from the same ingot, may greatly vary within the above limits as to the total amount of and as to the substances forming these impurities.

35 On the other hand, the amount and composition of such impurities even in case of such comparatively small amounts, greatly affect the crystalline structure of the aluminum and its behavior during etching.

40 Secondly, the grain structure of the aluminum and its reaction to etching is also dependent on variations in its heat treatment and working.

Thirdly, the surface condition of the aluminum, for example the degree of surface oxidation 45 and the amount of adhering impurities, also greatly affect the etching results, and while it is general practice to clean the aluminum surface prior to the etching, these effects are not fully eliminated and affect the etching of the aluminum surface.

50 All of the above factors contribute to cause the aluminum to etch at different rates under identical etching conditions.

Various attempts to check and control the etching, so as to get more uniform results have

been tried without finding an economic and satisfactory solution. While somewhat greater uniformity is obtained by using a very slow etching process, i. e., etching in low concentration solutions and at low temperatures, such slow etching, as it requires one or more hours, results in a poor utilization of the equipment, space, and labor, and is therefore uneconomical.

5 Therefore, in spite of the greater variations obtained, quick etching with high concentration 10 solutions and higher etching temperatures are used, with etching times running usually from one to five minutes.

15 My invention solves the above difficulties and provides for a very accurate control of the extent of etching of individual foils or electrodes, and results in a variation of usually less than  $\pm 10\%$ , and even less, of the capacity of the individual condensers made in accordance with any given specification.

20 My invention is of general utility for both slow and quick etching processes, and is of particular importance for quick etching processes where its superiority is particularly pronounced.

25 My invention is essentially a calorimetrically-controlled etching process, and is based on the realization that in etching aluminum an exothermic dissolution of the aluminum takes place whereby heat is liberated incidental to the reaction. As the amount of heat so liberated depends upon the amount of aluminum removed from the surface during the etching, the total amount of heat so liberated is a direct measure of the total amount of aluminum removed from the etched surface.

30 I have also found that the total amount of material removed from the etched aluminum indicates with considerable accuracy the extent of etching of the foil, provided the etching takes place under such conditions that the etching solution has a free and uniform access to all surface portions of the aluminum to be etched, and to some extent, that the volume of the etching solution is sufficiently large as to prevent during the 35 etching any important change in concentration of the etching solution.

One object of my invention is therefore to provide an etching process in which, by means of exact checking of the temperature rise of the 40 etching solution, the extent of the etching of the filming electrodes is controlled within very accurate limits.

45 A further object of my invention is to provide a quick etching process whereby the extent of etch-

5

10

15

20

25

30

35

40

45

50

55

ing is automatically indicated and controlled by the temperature rise of the etching solution.

A still further object of my invention is to provide an etching process by means of which, notwithstanding the usually occurring variations in the impurities of the filming metal, its grain structure, surface condition, etc., the extent of etching is kept closely uniform so that condensers having etched electrodes can be conveniently manufactured within capacity tolerances of  $\pm 10\%$  and even less.

Other objects of my invention will appear as the description progresses.

In the drawing forming part of this specification:

Figure 1 is a schematic diagram of an etching installation in accordance with the invention;

Fig. 2 is a perspective view of corrugated electrodes for wet electrolytic condensers stacked for etching;

Fig. 3 is a top view of two endless foils rolled together in a compact form for insertion in the etching bath.

Referring to Figure 1, the etching tank 1 is a container suitable to hold a sufficient amount of etching solution, for example 30 gallons for 5,000 to 10,000 square inches of aluminum surface to be simultaneously etched, and is made of a suitable material which is not attacked by the etching solution, for example glass, wood, stoneware, special stainless steels of the acid-resistant types, etc.

In practice, for reasons later to be stated, I usually prefer to use a metal tank.

The tank 1 contains a suitable etching solution 2, later to be specified. The aluminum to be etched, for example, the electrodes 3—3, after having been subjected to a suitable surface cleaning, for example by means of a weak alkaline solution, are immersed in the etching solution, for example by being placed on the supports 4—4, the supports being of a material which is not attacked by the etching solution.

Immersed in the etching bath is a mercury column thermometer 5. Two contact wires 6 and 7 are air-tightly sealed through the wall of the thermometer and so disposed that the contact 6 is always electrically connected through properly acid-proofly insulated leads with the mercury column 8 of the thermometer, whereas the mercury 8 only contacts with 7 when the etching bath has assumed a certain temperature, i. e., the one at which the etching is completed. The contacts 6 and 7 are connected in circuit in series with a battery 9 and a buzzer 10, which circuit is closed to sound a warning when the etching bath assumes the above referred to temperature.

It should be noted that the thermometer and the warning arrangement may be of any other suitable type; also, while I usually prefer to use such audible or visible warning device, such device can be dispensed with and observation of the thermometer left to the operator.

As stated before, the heat developed in the solution during the etching, and thus the temperature assumed by the etching solution (with certain corrections to be made and later referred to) gives a measure of the total amount of aluminum dissolved from the surface subjected to etching, and also with a very good degree of accuracy the extent of the etching of the foil.

The end temperature, i. e., the temperature at which the etching is completed, can be determined for any specific case either by computation or experimentally.

The computation of the end temperature of the etching solution is essentially a calorimetric computation, applied to the particular problem involved, and the general steps which I shall give below will suffice without further details to enable one skilled in the art to make such computations.

I first determine the heat capacity and total heat content of the etching solution at the starting temperature, i. e., at the temperature at which the aluminum to be etched is inserted into the solution.

After this I determine the volume and weight of aluminum to be removed by the etching. For this purpose I determine the total surface area of the aluminum exposed to the solution and the average depth of etching, i. e., the average thickness of the aluminum layer to be removed. I have found that within a fairly wide range of composition of the aluminum, there is a definite relationship between the average depth of etching and the so-called etching ratio. The latter ratio gives the increase of capacity of an etched electrode condenser compared with the capacity of an otherwise identical condenser using an unetched electrode. For example, to obtain an etching ratio of 5 it is necessary to etch to an average depth of about .007" measured from the surface of the aluminum.

After having determined the amount of aluminum to be removed, I compute the total amount of reaction heat liberated incidental to such removal. While the heat of reaction taking place in such removal of the aluminum somewhat varies with the etching solution used and the etching temperature, it is in average roughly about 150,000 calories per gram atom of aluminum.

The above total reaction heat raises the temperature of the etching bath, and the temperature is computed in known manner from the original heat content of the solution, the heat developed in the reaction and the heat capacity of the installation including the etching solutions, electrodes, supports, etc.

For exact computation certain corrections have to be made because of the heat losses due to conduction and radiation, and the variations in the specific heat of the etching solution with the temperature, etc.

As stated, instead of computing the desired final etching temperature I can determine it experimentally.

For the sake of greater uniformity, I prefer as a rule to start the etching operation always at a definite initial temperature of the etching solution, and for this reason I prefer to use a metal tank so that between the etching of consecutive batches of electrodes, the solution may be quickly cooled down to the same starting temperature, which I select as a rule somewhat above the prevailing room temperature.

While the metallic container increases the heat losses, correction can be conveniently made for such losses, and furthermore, because of the short etching times (I usually prefer to use 1 to 5 minutes) the heat losses in themselves are not necessarily important.

Sometimes, to permit a better utilization of the equipment, consecutive batches of electrodes are etched without permitting the solution to cool down to the same initial temperature. In such case, the change in heat of reaction and specific heat have to be compensated for various temperatures, and the predetermined temperature

rise or end temperature has to be determined for each particular starting temperature. This can again be done either experimentally or by computation.

In the arrangements above indicated the rise in temperature of the solution is usually of the order of 10° C. and for correct measurements I prefer to use alcohol or benzene thermometers.

As etching solution I may use various reagents, for example an aqueous solution of hydrochloric acid, the concentration of which depends primarily upon the desired etching time and etching temperature. In practice I use generally 5% to 20% solutions of hydrochloric acid, and use the lower concentrations for higher starting temperatures and/or longer etching times and vice versa.

For example, when starting etching at 25° C. and using an etching time of the order of one to five minutes (usually about three minutes) I use as a rule acid concentrations of 12% and 15%; whereas with higher starting temperatures, for example 35° C. and the above etching times, I prefer to use concentrations from 9% to 12%.

It should be noted that even fairly wide variations in concentration will not affect the accuracy of my process except that they may affect the duration thereof.

Instead of using hydrochloric acid solutions I may use a weak solution of hydrochloric acid together with salts of metallic chlorides, for example of nickel chloride, manganese chloride, copper chloride, and in some cases also sodium chloride. Furthermore, instead of hydrochloric acid other acids may be used, for example, trichloracetic acid, either alone or together with hydrochloric acid.

It should be noted that the free access of the etching solution to the electrode is of vital importance, as unless the solution has proper access to all surface portions of the aluminum, excessive temperature rises might occur locally in portions of the aluminum, which would result in uneven etching.

Thus the solution, besides having proper access to all portions of the aluminum for its proper etching, should also have free circulation for equal distribution of the heat and concentration. While artificial agitation of the etching solution can be provided for, as a rule this is unnecessary as a natural agitation takes place on account of the evolution of hydrogen gas which accompanies the etching process.

It should be noted that under certain circumstances a very high initial rate of etching may take place, which results in the formation of a gray to black deposit on the surface of the aluminum, which has an effect on the character of the etching.

The formation of such a deposit does not form part of this invention, and to obtain the usually desired results when such high rates of reaction are encountered accompanied by such black films, I prefer to interrupt the progress of the etching in the hydrochloric bath by removing the aluminum from this bath and immersing it into an alkaline solution, for example into a solution of sodium hydroxide. Such a treatment converts the black film on the surface of the aluminum into a white film, or removes it altogether; after this the aluminum may be reimmersed in the etching solution and the etching reaction allowed to proceed until the predetermined temperature rise is accomplished.

In carrying out this modification of my process,

the total temperature rise remains the same as if the etching had been uninterrupted. Thus in etching a batch of anodes where the predetermined temperature rise in the etching solution is from 25° C. to 35° C., I may interrupt the etching when the temperature reaches 28° C., and after treating the anodes in a caustic solution, replace them in the etching solution at 28° C., and then allow the temperature of the solution to reach 35° C.

When etching batches of corrugated or pleated electrodes, special measures may be necessary to assure proper access of the solution to all portions of the corrugations, and at the same time permit efficient utilization of the etching equipment. For example, when etching the pleated electrodes shown in Fig. 2, I stack batches of electrodes so that the longitudinal axes of successive electrodes are perpendicular to each other.

When etching foils of large lengths, for example so-called endless aluminum foils, and which after their etching are usually submitted to a continuous film-forming process according to the copending applications Ser. No. 548,270, filed July 1, 1931, and Ser. No. 741,493, filed August 25, 1934, of Preston Robinson, now respectively United States Patents Nos. 2,057,314 and 2,057,315, issued October 13, 1936, to make it possible to etch the foils in a compact form, I use an arrangement as indicated in Fig. 3, whereby two such foils 36 and 37 are wound into a coil. Thereby the foil 36 is corrugated, which insures the proper access and free circulation of the etching solution, whereas if a single flat foil or a single corrugated foil were wound into a roll proper access of the solution would not be insured.

After the etching has been performed, the corrugated foil 36 prior to film formation is preferably smoothed out by passing it through rolls, although with special forming equipment corrugated foils can also be properly filmed.

While I have described my invention in connection with specific examples and specific applications, I do not wish to be limited thereto, but desire the appended claims to be construed as broadly as permissible in view of the prior art.

What I claim is:

1. In the manufacture of electrolytic condensers, the process which comprises the steps, immersing aluminum electrodes in an etching bath comprising a 5% to 20% solution of hydrochloric acid, and removing the etched aluminum electrodes from the bath when the bath temperature, due to the heat developed by the exothermic reaction between said electrodes and said acid, has risen by a predetermined value above its initial value.

2. The process of manufacturing electrolytic condensers having etched electrodes with an etching ratio between 3 to 6, comprising the steps of subjecting the electrodes to etching for a duration of about 1 to 5 minutes, and controlling, by the amount of heat developed by the exothermic reaction of the etching, the extent of etching of the electrodes within a  $\pm 5\%$  to  $\pm 10\%$  accuracy.

3. In the manufacture of electrolytic condensers, the process which comprises, immersing filming electrodes in an acidic etching solution, interrupting said etching and placing said electrodes into an alkaline solution to remove undesirable deposits formed on said electrodes, and subsequently replacing the electrodes in said acidic solution to complete the etching.

4. In the manufacture of electrolytic con-

5       densers, the process which comprises, placing  
      filming electrodes in an acidic etching solution  
      having a predetermined initial temperature, in-  
      terrupting the etching and placing the electrodes  
      in an alkaline solution to remove undesirable  
      deposits formed on said electrodes, and subse-  
      quently replacing the electrodes in said etching  
      solution at the same solution temperature at  
      which the etching has been interrupted, and  
10      10     maintaining said electrodes in said etching solution  
      until the solution, in view of heat developed  
      by the exothermic reaction between said elec-  
      trodes and said solution, has assumed a prede-  
      termined temperature rise from its initial tem-  
15      15     perature.

20      5     In the manufacture of electrolytic con-  
      densers, the process which comprises, subjecting  
      in an etching solution filming electrodes to chem-  
      ical etching, measuring the temperature rise  
      caused by the exothermic reaction, and utilizing  
25      20     said temperature rise as an indicator of the de-  
      gree of etching.

25      6     In the manufacture of electrolytic con-  
      densers, the process of etching filming electrodes  
      comprising determining the amount of a given  
      electrode metal consumed by a given etching  
      solution in terms of the temperature rise of said  
      solution caused by the exothermic reaction be-  
30      30     tween said electrode metal and said solution dur-  
      ing the dissolution of a given amount of the  
      electrode metal, immersing an electrode of the  
      said metal in said etching solution, raising the  
      temperature of the etching solution by exothermic  
35      35     reaction between said electrode and said etching  
      solution, and interrupting the etching when said  
      etching solution has reached the predetermined  
      temperature corresponding to the amount of elec-  
      trode metal to be consumed in the etching process.

7. In the manufacture of electrolytic con-  
      densers, the process of etching aluminum elec-  
      trodes comprising determining the amount of alu-  
      minum consumed by a hydrochloric acid solu-  
      tion of a given concentration in terms of the  
      temperature rise of said solution caused by the  
      exothermic reaction between said aluminum and  
      said solution during the dissolution of a given  
      amount of the aluminum, immersing an aluminum  
      electrode in said solution, raising the tem-  
      perature of said solution by exothermic reaction  
      between the aluminum electrode and said solution,  
      measuring the temperature rise of the solution  
      due to said exothermic reaction, and inter-  
      rupting the etching at the point in the tempera-  
      ture rise of the solution which indicates the dis-  
      solution of the amount of aluminum of the elec-  
      trode sought to be dissolved in the etching  
      process.

8. In the etching of aluminum electrodes for  
      the manufacture of electrolytic condensers, the  
      process which comprises immersing an aluminum  
      electrode in a 5% to 20% solution of hydrochloric  
      acid at an initial temperature range of 25° C. to  
      45° C., raising the temperature of the etching  
      solution by the exothermic reaction between the  
      aluminum electrode and said solution, measuring  
      the temperature rise of the solution due to said  
      exothermic reaction, continuing the etching until  
      the heat generated by said exothermic reaction  
      has raised said etching solution from 5° C. to 15°  
      C. above its initial temperature, and interrupting  
      the etching at a point in the temperature rise  
      of from 5° C. to 15° C., which corresponds to the  
      measure of rise in temperature required to ob-  
      tain the desired degree of etching.

JOSEPH L. COLLINS.